

# UNITED STATES PATENT OFFICE.

RUDOLF FISCHER, OF STEGLITZ, GERMANY.

## PROCESS OF TONING PHOTOGRAPHIC SILVER-PICTURES.

1,079,756.

Specification of Letters Patent.

Patented Nov. 25, 1913.

No Drawing.

Application filed March 1, 1913. Serial No. 751,637.

*To all whom it may concern:*

Be it known that I, RUDOLF FISCHER, a citizen of the German Empire, and residing at Steglitz, near Berlin, Germany, have invented a certain new and useful Improved Process of Toning Photographic Silver-Pictures, of which the following is a specification.

My invention relates to a process of toning and intensifying photographic silver-pictures.

By the aid of suitable developers the latent picture in photographic layers can be developed directly into a colored picture in so far as the oxidation products, which are formed when the latent picture is reduced, are colored and, owing to their physical or chemical properties, remain at the place where they are formed. A yellowish-brown picture is so obtained when developing with pyrogallol, a blue picture with indoxyll, and a red one with thioindoxyll.

A primary object of my invention is to obtain colored pictures of this kind not from the latent picture, but from a black developed picture.

I have found that pictures which are developed black can be converted into colored pictures with developers of this kind by first converting the silver of such pictures into reducible silver compounds by a method known *per se*, *e. g.* by potassium ferricyanid and potassium bromid, and by then reducing such compounds with developers corresponding to requirements. In this case I obtain besides the silver picture a colored picture due to the colored oxidation product. In this manner it is possible subsequently to convert any black silver picture into a colored one. By repeating the operation new colored materials can be de-

posited at the places containing the silver, so that any desired intensification can be thereby obtained. Lastly, in order to obtain a pure colored picture the silver can be removed by one of the known reducing agents which will lighten the picture.

### *Example.*

50

1. A black silver picture is bleached in a solution of 10% potassium ferricyanid and 10% potassium bromid, well diluted with water and then developed to a yellowish-brown color in a solution of 0.1 g. pyrogallol, 2 g. sodium carbonate and 100 c. cm. of water.

55 2. A picture bleached as described in Example 1 is developed to a red color in a solution of 0.5 g. thioindoxyll carbonic acid, 5 c. cm. acetone, 2 g. potassium carbonate, and 100 c. cm. water.

I claim:—

60 1. The process of toning and intensifying photographic silver-pictures, consisting in first converting the silver in said pictures into reducible silver compounds, and then treating said compounds to produce oxidation products of the desired color.

65 2. The process of toning and intensifying photographic silver-pictures, consisting in first converting the silver in said pictures into reducible silver compounds, and then developing said pictures by developers adapted to convert said compounds into oxidation products of the desired color, said products remaining at the places where they are formed.

70 75 In testimony whereof, I affix my signature in the presence of two witnesses.

RUDOLF FISCHER.

Witnesses:

HENRY HASPER,  
WOLDEMAR HAUPT.